

[54] **CORROSION INHIBITOR FOR  
VANADIUM-CONTAINING FUELS**

[75] Inventors: Michael J. Zetlmeisl; Walter R. May; Robert R. Annand, all of St. Louis, Mo.

[73] Assignee: Petrolite Corporation, St. Louis, Mo.

[22] Filed: **Aug. 6, 1973**[21] Appl. No.: **386,228**[52] U.S. Cl. .... **44/51**; 44/67; 44/DIG. 3;  
252/387[51] Int. Cl. .... **C10L 1/32**; C10L 1/12; C10L 1/30[58] Field of Search..... **44/51, 67, DIG. 3;**  
252/387[56] **References Cited****UNITED STATES PATENTS**3,036,901 5/1962 Sanders et al. .... **44/67 X**  
3,628,925 12/1971 Milner ..... **44/51 X****FOREIGN PATENTS OR APPLICATIONS**

745,012 2/1956 United Kingdom

*Primary Examiner*—Delbert E. Gantz*Assistant Examiner*—I. Vaughn*Attorney, Agent, or Firm*—Sidney B. Ring; Hyman F. Glass

[57]

**ABSTRACT**

This invention relates to a composition containing calcium and aluminum, preferably in the ratio Ca/3Al, or calcium and aluminum in combination with Si, preferably in the ratio between about Ca/3Al/2Si and Ca/3Al/4Si (all calculated as metal weights); and to the use of such composition in petroleum fuels which contain vanadium, particularly in combination with sodium, for example in residual fuels so as to inhibit corrosion in the system, particularly in gas turbines. These compositions are superior to magnesium as an additive to such fuels, particularly in fuels which are high in sodium.

**10 Claims, 1 Drawing Figure**

COMPARISON OF ISOCORROSION LINES FOR VARIOUS ADDITIVE SYSTEMS (I CORR.  $\approx$   $\text{mA/cm}^2$ )

N.B.  $\text{SiO}_2$  AND  $\text{Al}_2\text{O}_3$  HAVE ONLY ONE POINT IN THE ACCEPTABLE RANGE AT THE CONCENTRATIONS OF  $\text{Na}$  AND  $\text{V}$  WHICH WERE TESTED.

## CORROSION INHIBITOR FOR VANADIUM-CONTAINING FUELS

The demand for greatly increased amounts of energy has forced utilities and other large-quantity users of fossil fuels to explore low-quality fuels for use in steam boilers and gas turbines. Fuels such as unrefined crude oil and residual oil contain large amounts of impurities which result in corrosive deposits in the equipment. Two of these impurities, sodium and vanadium, form 10 catastrophically corrosive, low melting slags that can destroy a vital part in a matter of hours.

Crude oil usually contains 1-500 ppm of vanadium in the form of a porphyrin complex depending on the source. Because of its origin as a concentrate from the refining process, residual oil contains several times more vanadium than the crude from which it was derived. The combustion of these vanadium-containing fuels produces very corrosive  $V_2O_5$  deposits which can 15 destroy a turbine part in a matter of days. Although the vanadium can be removed, the cost of the process cancels the economic advantage of using unrefined fuels. Vanadic corrosion is, therefore, usually controlled with chemical additives and optimization of operating conditions.

Sodium is almost always present in low-quality fuels, either directly in the crude oil or indirectly through contamination from various sources. The technology for removing sodium is well developed. These are limiting processes, however, and a trace of sodium must always be dealt with. For example, in maritime use the sodium level can be increased because of the introduction of sodium chloride through the air intake and contamination of the fuel by sea water. During combustion, the sodium reacts with the sulfur in the fuel to form the sulfate which is deposited in turbine parts. This reaction has been shown to be thermodynamically favored and results in the only sodium compound that will deposit under these conditions.

The mechanism of corrosion by vanadium and sodium has received much attention. Nascent oxygen species has been proposed as the corrosive active agent in  $V_2O_5$  melts. Various mechanisms have been presented to explain corrosive attack by sodium sulfate at metal surfaces. The classical method of inhibiting the corrosive characteristics of  $V_2O_5$  and  $Na_2SO_4$  melts has been to form high-melting vanadates of the former and minimize the level of the latter. Magnesium has been the most successful substance for this type of protection. The optimum levels of magnesium addition are not precisely known. Just as the mechanism of corrosion is only partially understood, so too is that of its inhibition.

There are other methods of limiting the corrosion such as reducing the operating temperature and maintaining the air to fuel ratio so that slightly reducing conditions exist during combustion. These types of methods may not be applicable. For example, the air to fuel ratio cannot be lowered to obtain reducing conditions in a gas turbine. Lower operating temperatures make the system less efficient and may be ruled out for economic reasons. Thus, chemical additives are often the best way to inhibit corrosion.

We have now discovered that certain combinations of metals synergistically inhibit fireside corrosion in gas turbines, steam boilers and furnaces. This invention comprises the addition of calcium and aluminum, or calcium and aluminum in combination with silicon, to

the fuels. We have discovered that Ca/Al additives are not only effective as compared to magnesium, the standard for the industry, but that Ca/Al also allows the fuel system to tolerate a sodium to vanadium ratio 10 times greater than when magnesium is employed.

We have further discovered that the use of silicon with Ca/Al further improves the system, particularly in view of the fact that it yields a slag which is more friable, water washable and more easily removed.

In practicing this invention, optimum results are achieved where the Ca/Al weight ratio is  $\frac{1}{2}$  calculated as metal weights. Although other ratios can be employed such as  $\frac{1}{2}$ , for example 1/2.5, and as low as  $\frac{1}{4}$ , the improvement of this invention is optimized at about the  $\frac{1}{2}$  ratio.

Where silicon is employed, the same ratios of Ca/Al inter se are employed with silicon added thereto. Optimum results are achieved where silicon is about 50% of the Ca/Al/Si mixture. Lesser amounts can also be employed such as where Si is as little as 1%, such as 25%, of the mixture, and as high as 99%, such as 75%, and preferably from 40 to 60%.

The corrosion rates of materials used in gas turbine, furnace and steam boiler construction in sodium-vanadium-sulfur containing slags may be determined by a variety of methods. The most reliable method is a field test in operating equipment. However, because of the costs involved, a variety of tests have been designed to either duplicate or reflect actual field conditions.

These range from high-pressure test rigs which are similar to gas turbines on a smaller scale to simple crucible tests carried out in a laboratory muffle furnace. We have developed an electrochemical technique for measuring corrosion rates in a laboratory scale furnace that accurately reflects the situation observed in larger test facilities and in the field. This technique is described in the article "High-Temperature Corrosion in Gas Turbines and Steam Boilers by Fuel Impurities. I. Measurement of Nickel Alloy Corrosion Rate in Molten Salts by Linear Polarization Technique," by Walter R. May, et al., *Industrial and Engineering Chemistry, Product Research and Development*, Vol. 11, No. 4, pg. 438, 1972. The data presented below in support of this disclosure was obtained by this

technique. Good correlation has been found between data from this test and field data. Data on magnesium are published in the articles "High-Temperature Corrosion in Gas Turbines and Steam Boilers by Fuel Impurities. II. The Sodium Sulfate-Magnesium Sulfate-Vanadium Pentoxide System" and "III. Evaluation of Magnesium as a Corrosion Inhibitor," *Industrial and Engineering Chemistry*, Vol. 12, No. 2, pgs. 140-149, 1973.

Corrosion rate data taken in this manner on the  $Na_2SO_4-CaSO_4-Al_2O_3-V_2O_5$  system are presented in Table I. For comparison, similar data for magnesium are presented in Table II.

From these data, it can easily be seen that in the calcium-aluminum system, the Na/V ratio can be tolerated at 10 times the level for the magnesium system. For example, compare Mg/V=4 and Na/V=0.1 in Table II with Ca/V=0.79, Al/V=3 and Na/V=1 in Table I. At 900°C., corrosion currents of 0.0438 mg/in.-hr. were obtained for aluminum-calcium whereas 0.230 mg/in.-hr. was obtained in the magnesium system. We considered 0.05 mg/in.-hr., which corresponds to 10 mpy for Udimet 500, the maximum permitted corrosion rate. A similar table of data are presented in Table

III for the calcium-aluminum-silicon system. From these data, the FIGURE of this invention was drawn.

Table I

| Na/V  | Ratio<br>Ca/V | Al/V  | Corrosion Rates for Udimet 500<br>in Various $\text{Na}_2\text{SO}_4$ — $\text{CaSO}_4$ — $\text{SiO}_2$ — $\text{Al}_2\text{O}_3$ — $\text{V}_2\text{O}_5$ Compositions |                 |                         |                        |       | 'corr(ma/cm²)* |       |       |     |
|-------|---------------|-------|--------------------------------------------------------------------------------------------------------------------------------------------------------------------------|-----------------|-------------------------|------------------------|-------|----------------|-------|-------|-----|
|       |               |       | Mole Percent                                                                                                                                                             |                 |                         |                        |       | 800            | 850   | 900   | 950 |
|       |               |       | $\text{Na}_2\text{SO}_4$                                                                                                                                                 | $\text{CaSO}_4$ | $\text{Al}_2\text{O}_3$ | $\text{V}_2\text{O}_5$ |       |                |       |       |     |
| 1     | 0.79          | 1     | 31.15                                                                                                                                                                    | 28.26           | 26.54                   | 14.05                  | 16.4  | 17.3           | 26.7  | 35.3  |     |
| 1     | 1.58          | 1     | 24.29                                                                                                                                                                    | 44.07           | 20.70                   | 10.95                  | —     | —              | 37.2  | 54.8  |     |
| 1     | 0.79          | 2     | 24.62                                                                                                                                                                    | 22.33           | 41.95                   | 11.10                  | .768  | 1.14           | 1.82  | 2.79  |     |
| 1     | 1.58          | 2     | 20.12                                                                                                                                                                    | 36.51           | 34.29                   | 9.07                   | .891  | 1.78           | 3.01  | 4.13  |     |
| 1     | 0.79          | 3     | 20.35                                                                                                                                                                    | 18.46           | 52.02                   | 9.17                   | 5.56  | 6.95           | 9.73  | 14.4  |     |
| 1     | 2.37          | 1     | 19.90                                                                                                                                                                    | 54.16           | 16.96                   | 8.97                   | 3.67  | 6.73           | 11.6  | 20.2  |     |
| 1     | 1.58          | 3     | 17.18                                                                                                                                                                    | 31.17           | 43.91                   | 7.75                   | .303  | .440           | .586  | .879  |     |
| 1     | 2.37          | 2     | 17.02                                                                                                                                                                    | 46.31           | 29.00                   | 7.67                   | .74   | 1.0            | 1.66  | 2.35  |     |
| 1     | 2.37          | 3     | 14.86                                                                                                                                                                    | 40.45           | 37.99                   | 6.70                   | .263  | .323           | .404  | .404  |     |
| 1     | 0.23          | 0.72  | 41.92                                                                                                                                                                    | 13.46           | 25.72                   | 18.90                  | 14.28 | 17.8           | 20.3  | 24.2  |     |
| 1     | 0.56          | 1.44  | 22.38                                                                                                                                                                    | 40.06           | 27.46                   | 10.09                  | 2.21  | 2.80           | 5.9   | 12.3  |     |
| 1     | 0.84          | 2.16  | 23.50                                                                                                                                                                    | 22.65           | 43.25                   | 10.60                  | 1.69  | 3.98           | 4.94  | 6.78  |     |
| 1     | 1.12          | 2.88  | 19.27                                                                                                                                                                    | 24.76           | 47.28                   | 8.69                   | .522  | 1.42           | 1.86  | 2.39  |     |
| 1     | 1.40          | 3.60  | 16.33                                                                                                                                                                    | 26.22           | 50.09                   | 7.36                   | 1.41  | 2.75           | 3.57  | 4.98  |     |
| 1     | 2.80          | 7.20  | 9.26                                                                                                                                                                     | 29.75           | 56.82                   | 4.18                   | .0206 | .0374          | .0975 | .167  |     |
| 1     | 5.60          | 14.40 | 4.96                                                                                                                                                                     | 31.89           | 60.91                   | 2.24                   | .0393 | .0524          | .0655 | .0712 |     |
| 1     | 8.4           | 21.6  | 3.39                                                                                                                                                                     | 32.68           | 62.41                   | 1.53                   | .0398 | .0507          | .0602 | .0708 |     |
| 1     | 11.2          | 28.8  | 2.57                                                                                                                                                                     | 33.03           | 63.18                   | 1.16                   | .0267 | .032           | .0533 | .056  |     |
| 1     | 14.0          | 36.0  | 2.08                                                                                                                                                                     | 33.33           | 63.66                   | 0.94                   | .0160 | .0173          | .0240 | .0267 |     |
| 0.1   | 0.79          | 1     | 4.33                                                                                                                                                                     | 39.27           | 36.88                   | 19.52                  | .246  | .325           | .396  | .476  |     |
| 0.1   | 1.58          | 1     | 3.11                                                                                                                                                                     | 56.39           | 26.48                   | 14.01                  | .153  | .223           | .282  | .388  |     |
| 0.1   | 0.79          | 2     | 3.16                                                                                                                                                                     | 28.69           | 53.89                   | 14.26                  | .0206 | .0311          | .0362 | .0621 |     |
| 0.1   | 1.58          | 2     | 2.46                                                                                                                                                                     | 44.58           | 41.88                   | 11.08                  | .0177 | .0442          | .0618 | .0973 |     |
| 0.1   | 0.79          | 3     | 2.49                                                                                                                                                                     | 22.60           | 63.68                   | 11.23                  | .035  | .0524          | .0438 | .0874 |     |
| 0.1   | 2.37          | 1     | 2.42                                                                                                                                                                     | 65.98           | 20.66                   | 10.93                  | .0516 | .0688          | .124  | .206  |     |
| 0.1   | 1.58          | 3     | 2.03                                                                                                                                                                     | 36.87           | 51.94                   | 9.16                   | .0115 | .0345          | .0574 | .0688 |     |
| 0.1   | 2.37          | 2     | 2.01                                                                                                                                                                     | 54.69           | 34.24                   | 9.06                   | .0208 | .0249          | .0332 | .0457 |     |
| 0.1   | 2.37          | 3     | 1.71                                                                                                                                                                     | 46.76           | 43.80                   | 7.73                   | .0115 | .0087          | .0115 | .0232 |     |
| 0.01  | 0.79          | 1     | 0.45                                                                                                                                                                     | 40.86           | 38.38                   | 20.31                  | 1.04  | 1.51           | 1.67  | 1.98  |     |
| 0.01  | 1.58          | 1     | 0.32                                                                                                                                                                     | 58.02           | 27.25                   | 14.42                  | .042  | .053           | .111  | .126  |     |
| 0.01  | 0.79          | 2     | 0.33                                                                                                                                                                     | 29.53           | 55.47                   | 14.68                  | .0243 | .0388          | .0630 | .0873 |     |
| 0.01  | 1.58          | 2     | 0.25                                                                                                                                                                     | 45.59           | 42.83                   | 11.33                  | .0138 | .0166          | .0221 | .0276 |     |
| 0.01  | 0.79          | 3     | 0.25                                                                                                                                                                     | 23.12           | 65.14                   | 11.49                  | .0357 | .0536          | .0714 | .119  |     |
| 0.01  | 2.37          | 1     | 0.25                                                                                                                                                                     | 67.46           | 21.12                   | 11.18                  | .074  | .108           | .133  | .207  |     |
| 0.01  | 1.58          | 3     | 0.21                                                                                                                                                                     | 37.55           | 52.91                   | 9.33                   | .0192 | .0240          | .0335 | .0478 |     |
| 0.01  | 2.37          | 2     | 0.20                                                                                                                                                                     | 55.69           | 34.87                   | 9.23                   | .0084 | .0126          | .0210 | .0335 |     |
| 0.01  | 2.37          | 3     | 0.17                                                                                                                                                                     | 47.42           | 44.54                   | 7.86                   | .0088 | .0131          | .0175 | .0526 |     |
| 0.001 | 0.79          | 1     | 0.05                                                                                                                                                                     | 41.03           | 38.54                   | 20.39                  | 1.35  | 1.81           | 2.32  | 2.92  |     |
| 0.001 | 1.58          | 1     | 0.03                                                                                                                                                                     | 58.18           | 27.33                   | 14.46                  | .257  | .322           | .354  | .386  |     |
| 0.001 | 0.79          | 2     | 0.03                                                                                                                                                                     | 29.61           | 55.63                   | 14.72                  | .054  | .049           | .081  | .086  |     |
| 0.001 | 1.58          | 2     | 0.03                                                                                                                                                                     | 45.70           | 42.92                   | 11.36                  | .085  | .058           | .044  | .041  |     |
| 0.001 | 0.79          | 3     | 0.03                                                                                                                                                                     | 23.17           | 65.29                   | 11.52                  | .0047 | .0071          | .0094 | .024  |     |
| 0.001 | 2.37          | 1     | 0.02                                                                                                                                                                     | 67.61           | 21.17                   | 11.20                  | .349  | .436           | .653  | .828  |     |
| 0.001 | 1.58          | 3     | 0.02                                                                                                                                                                     | 37.62           | 53.01                   | 9.35                   | .096  | .036           | .0598 | .0683 |     |
| 0.001 | 2.37          | 2     | 0.02                                                                                                                                                                     | 55.80           | 34.94                   | 9.24                   | .0276 | .0328          | .0493 | .0766 |     |
| 0.001 | 2.37          | 3     | 0.02                                                                                                                                                                     | 47.50           | 44.62                   | 7.87                   | .0396 | .0509          | .0736 | .125  |     |

\*Some of the corrosion rate data are given as corrosion currents (ma/cm²) and some as corrosion rates (mg/cm²-hr). The conversion from corrosion current to corrosion rate for Udimet 500 is 0.95. Within the experimental limitations of the procedure, the two values can be considered identical.

Table II

| Na <sub>2</sub> SO <sub>4</sub> | MgSO <sub>4</sub> | V <sub>2</sub> O <sub>5</sub> | Wt ratio | Corrosion Rate for Udimet 500 in Various $\text{Na}_2\text{SO}_4$ — $\text{MgSO}_4$ — $\text{V}_2\text{O}_5$ Compositions from 800° to 950° |        |        |        |        |
|---------------------------------|-------------------|-------------------------------|----------|---------------------------------------------------------------------------------------------------------------------------------------------|--------|--------|--------|--------|
|                                 |                   |                               |          | Na/V                                                                                                                                        | 800°   | 850°   | 900°   | 950°   |
| 34.056                          | 64.408            | 1.535                         | 10       | 10                                                                                                                                          | 0.408  | 0.533  | 0.941  | 1.76   |
| 20.714                          | 78.352            | 0.934                         | 20       | 10                                                                                                                                          | 0.581  | 1.09   | 1.38   | 2.98   |
| 14.884                          | 84.445            | 0.671                         | 30       | 10                                                                                                                                          | 0.283  | 0.571  | 0.835  | 1.45   |
| 11.614                          | 87.862            | 0.524                         | 40       | 10                                                                                                                                          | 0.723  | 1.11   | 1.78   | 3.23   |
| 9.523                           | 90.050            | 0.429                         | 50       | 10                                                                                                                                          | 0.274  | 0.768  | 1.34   | 2.12   |
| 5.010                           | 94.763            | 0.226                         | 100      | 10                                                                                                                                          | 0.684  | 1.10   | 1.83   | 2.37   |
| 2.572                           | 97.311            | 0.116                         | 200      | 10                                                                                                                                          | 0.211  | 0.341  | 0.578  | 0.675  |
| 1.730                           | 98.191            | 0.0781                        | 300      | 10                                                                                                                                          | 0.0291 | 0.117  | 0.167  | 0.247  |
| 1.303                           | 98.637            | 0.0588                        | 400      | 10                                                                                                                                          | 0.0154 | 0.0760 | 0.149  | 0.184  |
| 0.951                           | 99.005            | 0.0430                        | 500      | 10                                                                                                                                          | 0.0154 | 0.0257 | 0.0361 | 0.102  |
| 29.918                          | 56.581            | 13.502                        | 1        | 1                                                                                                                                           | 17.8   | 14.0   | 24.7   | 26.1   |
| 19.106                          | 72.271            | 8.623                         | 2        | 1                                                                                                                                           | 11.8   | 25.8   | 29.6   | 29.6   |
| 14.035                          | 79.631            | 8.334                         | 3        | 1                                                                                                                                           | 2.30   | 2.48   | 3.12   | 4.87   |
| 11.09                           | 83.90             | 5.01                          | 4        | 1                                                                                                                                           | 2.55   | 3.67   | 4.62   | 5.22   |
| 9.168                           | 86.694            | 4.137                         | 5        | 1                                                                                                                                           | 2.98   | 3.67   | 3.67   | 9.70   |
| 4.911                           | 92.875            | 2.214                         | 10       | 1                                                                                                                                           | 0.214  | 0.314  | 0.536  | 1.54   |
| 2.546                           | 96.306            | 1.148                         | 20       | 1                                                                                                                                           | 0.056  | 0.092  | 0.154  | 0.400  |
| 1.719                           | 97.507            | 0.775                         | 30       | 1                                                                                                                                           | 0.039  | 0.0833 | 0.0985 | 0.138  |
| 1.297                           | 98.118            | 0.585                         | 40       | 1                                                                                                                                           | 0.0137 | 0.0165 | 0.0219 | 0.0820 |
| 1.042                           | 98.488            | 0.470                         | 50       | 1                                                                                                                                           | 0.0185 | 0.0185 | 0.0258 | 0.048  |
| 4.094                           | 77.429            | 18.477                        | 1        | 0.1                                                                                                                                         | 0.290  | 1.74   | 3.20   | 3.48   |
| 2.307                           | 87.279            | 10.413                        | 2        | 0.1                                                                                                                                         | 0.163  | 0.785  | 1.58   | 1.58   |
| 1.606                           | 91.144            | 7.250                         | 3        | 0.1                                                                                                                                         | 0.0358 | 1.45   | 1.80   | 2.57   |
| 1.23                            | 93.21             | 5.56                          | 4        | 0.1                                                                                                                                         | 0.0673 | 1.35   | 0.230  | 0.379  |
| 0.999                           | 94.495            | 4.506                         | 5        | 0.1                                                                                                                                         | 0.023  | 0.258  | 0.371  | 0.387  |
| 0.514                           | 97.170            | 2.317                         | 10       | 0.1                                                                                                                                         | 0.349  | 0.392  | 0.491  | 1.03   |
| 0.261                           | 98.565            | 1.175                         | 20       | 0.1                                                                                                                                         | 0.0898 | 0.0943 | 0.123  | 0.151  |
| 0.175                           | 99.038            | 0.787                         | 30       | 0.1                                                                                                                                         | 0.054  | 0.033  | 0.043  | 0.035  |

Table II-continued

| Corrosion Rate for Udimet 500 in Various $\text{Na}_2\text{SO}_4$ — $\text{MgSO}_4$ — $\text{V}_2\text{O}_5$ Compositions from 800 to 950° |                 |                        |      | Corrosion rate, mg/cm² hr |         |         |         |
|--------------------------------------------------------------------------------------------------------------------------------------------|-----------------|------------------------|------|---------------------------|---------|---------|---------|
| Mol %                                                                                                                                      |                 | Wt ratio               |      | 800°                      | 850°    | 900°    | 950°    |
| $\text{Na}_2\text{SO}_4$                                                                                                                   | $\text{MgSO}_4$ | $\text{V}_2\text{O}_5$ | Mg/V | Na/V                      |         |         |         |
| 0.425                                                                                                                                      | 80.39           | 19.18                  | 1    | 0.01                      | 0.162   | 0.261   | 0.349   |
| 0.236                                                                                                                                      | 89.13           | 10.63                  | 2    | 0.01                      | 0.129   | 0.189   | 0.324   |
| 0.163                                                                                                                                      | 92.48           | 7.36                   | 3    | 0.01                      | 0.0351  | 0.0432  | 0.0674  |
| 0.125                                                                                                                                      | 94.25           | 5.62                   | 4    | 0.01                      | 0.0290  | 0.0172  | 0.0319  |
| 0.101                                                                                                                                      | 95.35           | 4.55                   | 5    | 0.01                      | 0.00324 | 0.00665 | 0.00640 |
| 0.0427                                                                                                                                     | 80.700          | 19.257                 | 1    | 0.001                     | 0.998   | 1.81    | 3.22    |
| 0.0236                                                                                                                                     | 89.319          | 10.657                 | 2    | 0.001                     | 0.0136  | 0.0136  | 0.152   |
| 0.0163                                                                                                                                     | 92.617          | 7.367                  | 3    | 0.001                     | 0.0350  | 0.0275  | 0.0418  |
| 0.01                                                                                                                                       | 94.36           | 5.63                   | 4    | 0.001                     | 0.0130  | 0.0161  | 0.0276  |
| 0.0101                                                                                                                                     | 95.435          | 4.555                  | 5    | 0.001                     | 0.00722 | 0.0144  | 0.0289  |
| 0.50                                                                                                                                       | 99.50           | 0.00                   |      |                           | 0.0127  | 0.0190  | 0.0169  |
| 1.00                                                                                                                                       | 99.00           | 0.00                   |      |                           | 0.0116  | 0.162   | 0.196   |
| 5.00                                                                                                                                       | 95.00           | 0.00                   |      |                           | 0.157   | 0.755   | 1.05    |
| 10                                                                                                                                         | 90              | 0                      |      |                           |         | 1.71    | 1.99    |
| 25                                                                                                                                         | 75              | 0                      |      |                           | 0.552   | 1.01    | 1.39    |
| 33.3                                                                                                                                       | 66.7            | 0                      |      |                           | 1.06    | 1.76    | 2.51    |
| 50                                                                                                                                         | 50              | 0                      |      |                           | 1.56    | 2.59    | 3.62    |
| 75                                                                                                                                         | 25              | 0                      |      |                           | 1.39    | 1.95    | 4.43    |
| 90                                                                                                                                         | 10              | 0                      |      |                           | 0.567   | 0.957   | 2.18    |
| 100                                                                                                                                        | 0               | 0                      |      |                           | 0.361   | 0.542   | 0.794   |
| 0                                                                                                                                          | 90              | 10                     | 2.45 | 0                         | 0.0382  | 0.0607  | 0.101   |
| 0                                                                                                                                          | 80              | 20                     | 0.95 | 0                         | 0.557   | 0.835   | 0.932   |
| 0                                                                                                                                          | 70              | 30                     | 0.56 | 0                         | 0.340   | 0.483   | 0.727   |
| 0                                                                                                                                          | 60              | 40                     | 0.36 | 0                         | 25.8    | 44.8    | 89.8    |
| 90                                                                                                                                         | 0               | 10                     | 0    | 4.06                      | 20.0    | 25.0    | 22.7    |
| 80                                                                                                                                         | 0               | 20                     | 0    | 1.81                      | 28.6    | 30.9    | 34.3    |
| 75                                                                                                                                         | 0               | 25                     | 0    | 1.35                      | 23.8    | 28.9    | 40.7    |
| 66.7                                                                                                                                       | 0               | 33.3                   | 0    | 0.90                      | 36.4    | 38.1    | 47.3    |
| 50                                                                                                                                         | 0               | 50                     | 0    | 0.45                      | 73.5    | 81.8    | 89.8    |
| 14.3                                                                                                                                       | 0               | 85.7                   | 0    | 0.075                     | 65.8    | 94.8    | 107     |
| 0                                                                                                                                          | 0               | 100                    |      |                           | 32.2    | 59.3    | 79.3    |
|                                                                                                                                            |                 |                        |      |                           |         |         | 191     |

Table III

| Corrosion Rates for Udimet 500<br>in Various $\text{Na}_2\text{SO}_4$ — $\text{CaSO}_4$ — $\text{SiO}_2$ — $\text{Al}_2\text{O}_3$ — $\text{V}_2\text{O}_5$ Compositions |      |      |      |                          |                 |                |                         |                        |        |        |       |       |
|--------------------------------------------------------------------------------------------------------------------------------------------------------------------------|------|------|------|--------------------------|-----------------|----------------|-------------------------|------------------------|--------|--------|-------|-------|
| Ratio                                                                                                                                                                    |      |      |      | Mole Percent             |                 |                |                         |                        |        |        |       |       |
| Na/V                                                                                                                                                                     | Ca/V | Si/V | Al/V | $\text{Na}_2\text{SO}_4$ | $\text{CaSO}_4$ | $\text{SiO}_2$ | $\text{Al}_2\text{O}_3$ | $\text{V}_2\text{O}_5$ | 800°   | 850°   | 900°  | 950°  |
| 1                                                                                                                                                                        | 1    | 1    | 1    | 19.655                   | 22.549          | 32.178         | 16.748                  | 8.870                  | 1.99   | 3.80   | 6.52  | 9.23  |
| 1                                                                                                                                                                        | 2    | 1    | 1    | 16.039                   | 36.800          | 26.257         | 13.666                  | 7.238                  | 3.75   | 5.63   | 8.36  | 15.18 |
| 1                                                                                                                                                                        | 1    | 2    | 1    | 14.870                   | 17.059          | 48.689         | 12.670                  | 6.711                  | .623   | .917   | 1.51  | 2.01  |
| 1                                                                                                                                                                        | 1    | 1    | 2    | 16.836                   | 19.314          | 27.562         | 28.690                  | 7.598                  | .277   | .501   | .983  | 1.37  |
| 1                                                                                                                                                                        | 2    | 2    | 1    | 12.703                   | 29.146          | 41.593         | 10.824                  | 5.733                  | .859   | 1.38   | 2.28  | 2.54  |
| 1                                                                                                                                                                        | 2    | 1    | 2    | 14.111                   | 32.375          | 23.100         | 24.046                  | 6.368                  | .093   | .170   | .266  | .368  |
| 1                                                                                                                                                                        | 1    | 2    | 2    | 13.198                   | 15.141          | 43.213         | 22.491                  | 5.956                  | .0145  | .027   | .029  | .228  |
| 1                                                                                                                                                                        | 2    | 2    | 2    | 11.463                   | 26.300          | 37.531         | 19.534                  | 5.173                  | .149   | .166   | .236  | .323  |
| 0.1                                                                                                                                                                      | 1    | 1    | 1    | 2.388                    | 27.395          | 39.094         | 20.347                  | 10.777                 | .24    | .32    | .37   | .40   |
| 0.1                                                                                                                                                                      | 2    | 1    | 1    | 1.874                    | 43.008          | 30.687         | 15.972                  | 8.459                  | .626   | .793   | .834  | .876  |
| 0.1                                                                                                                                                                      | 1    | 2    | 1    | 1.717                    | 19.695          | 56.212         | 14.628                  | 7.748                  | .0195  | .0226  | .0329 | .0534 |
| 0.1                                                                                                                                                                      | 1    | 1    | 2    | 1.984                    | 22.763          | 32.484         | 33.814                  | 8.955                  | .0180  | .0235  | .0271 | .0307 |
| 0.1                                                                                                                                                                      | 2    | 2    | 1    | 1.434                    | 32.909          | 46.963         | 12.221                  | 6.473                  | .109   | .143   | .176  | .193  |
| 0.1                                                                                                                                                                      | 2    | 1    | 2    | 1.616                    | 37.085          | 26.461         | 27.544                  | 7.294                  | .0573  | .0823  | .107  | .129  |
| 0.1                                                                                                                                                                      | 1    | 2    | 2    | 1.498                    | 17.182          | 49.638         | 25.523                  | 6.759                  | .0184  | .0258  | .0268 | .0478 |
| 0.1                                                                                                                                                                      | 2    | 2    | 2    | 1.278                    | 29.325          | 41.848         | 21.781                  | 5.768                  | .0250  | .0293  | .0368 | .0498 |
| 0.01                                                                                                                                                                     | 1    | 1    | 1    | 0.244                    | 27.996          | 39.952         | 20.794                  | 11.013                 | .0643  | .0643  | .0643 | .0944 |
| 0.01                                                                                                                                                                     | 2    | 1    | 1    | 0.191                    | 43.746          | 31.214         | 16.246                  | 8.605                  | .0367  | .0496  | .0648 | .0906 |
| 0.01                                                                                                                                                                     | 1    | 2    | 1    | 0.174                    | 20.004          | 57.094         | 14.857                  | 7.869                  | .0231  | .0370  | .0703 | .0795 |
| 0.01                                                                                                                                                                     | 1    | 1    | 2    | 0.202                    | 23.177          | 33.075         | 34.429                  | 9.118                  | .0042  | .0053  | .0084 | .0148 |
| 0.01                                                                                                                                                                     | 2    | 2    | 1    | 0.145                    | 33.339          | 47.577         | 12.381                  | 6.558                  | .0218  | .0294  | .0348 | .0533 |
| 0.01                                                                                                                                                                     | 2    | 1    | 2    | 0.164                    | 37.632          | 26.851         | 27.951                  | 7.402                  | .0218  | .0283  | .0468 | .0698 |
| 0.01                                                                                                                                                                     | 1    | 2    | 2    | 0.152                    | 17.417          | 49.708         | 25.872                  | 6.851                  | .002   | .002   | .003  | .0042 |
| 0.001                                                                                                                                                                    | 2    | 2    | 2    | 0.129                    | 29.666          | 42.335         | 22.034                  | 5.835                  | .0109  | .0153  | .0174 | .0218 |
| 0.001                                                                                                                                                                    | 1    | 1    | 1    | 0.024                    | 28.058          | 40.040         | 20.840                  | 11.038                 | .0717  | .0942  | .127  | .156  |
| 0.001                                                                                                                                                                    | 2    | 1    | 1    | 0.019                    | 43.821          | 31.267         | 16.274                  | 8.619                  | .0235  | .0326  | .0428 | .0612 |
| 0.001                                                                                                                                                                    | 1    | 2    | 1    | 0.017                    | 20.036          | 57.184         | 14.881                  | 7.882                  | .0117  | .0117  | .0117 | .0176 |
| 0.001                                                                                                                                                                    | 1    | 1    | 2    | 0.020                    | 23.219          | 33.135         | 34.491                  | 9.134                  | .0089  | .0133  | .0192 | .0258 |
| 0.001                                                                                                                                                                    | 2    | 2    | 1    | 0.015                    | 33.383          | 47.639         | 12.397                  | 6.566                  | .0324  | .0392  | .0579 | .0682 |
| 0.001                                                                                                                                                                    | 2    | 1    | 2    | 0.016                    | 37.688          | 26.891         | 27.992                  | 7.413                  | .0235  | .0326  | .0428 | .0612 |
| 0.001                                                                                                                                                                    | 1    | 2    | 2    | 0.015                    | 17.440          | 49.776         | 25.907                  | 6.801                  | .00033 | .00131 | .0033 | .0033 |
| 0.001                                                                                                                                                                    | 2    | 2    | 2    | 0.013                    | 29.701          | 42.384         | 22.060                  | 5.842                  | .0022  | .0025  | .0025 | .0031 |

-continued

For Ca/3 Al/2 Si: parts additive=3[V]+15[Na]

The following series of equations approximate the amount of additive to be employed at 900°C. All values for the additives and metal weights are in ppm.

For Mg: parts additive=4[V]+40[Na]  
 For Mg/Si: parts additive=8[V]+80[Na]  
 For Ca/3 Al: parts additive=3[V]+15[Na]

65 Note the following. First, these equations will give only a fairly close approximation of the required dosage. Secondly, the equations seem to work for high vanadium levels only when the sodium levels are also

fairly high. Since such high vanadium-sodium levels will be seldom encountered, if ever, fitting the data for lower vanadium levels is clearly more useful.

In practice, for fuels containing low vanadium, i.e., V up to 12 ppm and Na up to 5 ppm, one employs up to 100 ppm of the additives of this invention, such as to 80 ppm, but preferably no more than 70 ppm.

When the fuels contain high vanadium, i.e., V over 12 ppm and Na up to 5 ppm, one employs about 50 to 2500 ppm, such as from about 70 to 2000 ppm but preferably from about 100 to 1500 ppm.

The superiority of the present invention is graphically presented in the FIGURE of this invention where additive/V is plotted against Na/V, so as to yield isocorrosion lines, i.e., 99.9% protection. The superiority of the additives of the present invention over magnesium, the standard additive for the industry, is clearly illustrated in this FIGURE.

From these equations and the FIGURE, Table IV was constructed to demonstrate the superiority of the calcium-aluminum and calcium-aluminum-silicon additives over magnesium.

Table IV

| Crude                     | V(ppm)  | Na Level(ppm) | Dosage for Particular Crude Oils<br>Containing Vanadium at Several Na Levels |                  |                |
|---------------------------|---------|---------------|------------------------------------------------------------------------------|------------------|----------------|
|                           |         |               | Mg                                                                           | Mg + Si          | Additive (ppm) |
|                           |         |               | Ca - 3 Al                                                                    | Ca - 3 Al - 2 Si |                |
| Abu Dhabi<br>(Mid East)   | <1-1.5  | .05           | 8-9                                                                          | 13-15            | 3.6-5          |
|                           |         | .15           | 13-15                                                                        | 25               | 5-7            |
|                           |         | .5            | 23-30                                                                        | 60               | 10-11          |
|                           |         | 1.5           | 60                                                                           | 150              | 22-24          |
|                           |         | 5             | 150-200                                                                      | ≈300             | 70             |
| Arabian Light             | 12      | .05           | 36                                                                           | 57.6             | 31.2           |
|                           |         | .15           | 54                                                                           | 84               | 32.4           |
|                           |         | .5            | 77                                                                           | 144              | 40.8           |
|                           |         | 1.5           | 144                                                                          | 252              | 60             |
|                           |         | 5             | 300                                                                          | 600              | 108            |
| East Texas<br>Cretaceous  | 4       | .05           | 17                                                                           | 28               | 10             |
|                           |         | .15           | 28                                                                           | 44               | 10.4           |
|                           |         | .5            | 48                                                                           | 84               | 12.8           |
|                           |         | 1.5           | 92                                                                           | 224              | 16.8           |
|                           |         | 5             | 220                                                                          | 480              | 32             |
| Bachaquero<br>(Venezuela) | 413     | .05           | ≈450                                                                         | 1280             | 1033           |
|                           |         | .15           | 620                                                                          | 1404             | 1033           |
|                           |         | .5            | 826                                                                          | 1652             | 1033           |
|                           |         | 1.5           | 1074                                                                         | 1900             | 1033           |
|                           |         | 5             | 1735                                                                         | 2891             | 1115           |
| Boscan<br>(Venezuela)     | 900     | .05           | ≈900                                                                         | ≈2700            | 2250           |
|                           |         | .15           | 1080                                                                         | 2880             | 2250           |
|                           |         | .5            | 1530                                                                         | 3240             | 2250           |
|                           |         | 1.5           | 1980                                                                         | 3600             | 2250           |
|                           |         | 5             | 2880                                                                         | 4500             | 2340           |
| El Alamein<br>(Egypt)     | 15      | .05           | 39                                                                           | 67.5             | 37.5           |
|                           |         | .15           | 60                                                                           | 94.5             | 37.5           |
|                           |         | .5            | 97.5                                                                         | 150              | 46.5           |
|                           |         | 1.5           | 165                                                                          | 270              | 66             |
|                           |         | 5             | 315                                                                          | 600              | 113            |
| Gabon<br>(Africa)         | 4-10    | .05           | 18-31                                                                        | 28-50            | 11-26          |
|                           |         | .15           | 28-48                                                                        | 44-70            | 13-28          |
|                           |         | .5            | 48-80                                                                        | 84-120           | 19-34          |
|                           |         | 1.5           | 104-130                                                                      | 184-230          | 32-50          |
|                           |         | 5             | 260-270                                                                      | 500-600          | 76-100         |
| Kuwait<br>(Neutral Zone)  | 60      | .05           | 108                                                                          | 228              | 150            |
|                           |         | .15           | 360                                                                          | 258              | 150            |
|                           |         | .5            | 228                                                                          | 360              | 150            |
|                           |         | 1.5           | 360                                                                          | 540              | 180            |
|                           |         | 5             | 600                                                                          | 960              | 240            |
| Libya,<br>Es Sider        | 2.5     | .05           | 13                                                                           | 20               | 7.5            |
|                           |         | .15           | 22                                                                           | 34               | 9.5            |
|                           |         | .5            | 40                                                                           | 45               | 15             |
|                           |         | 1.5           | 45                                                                           | 163              | 27.5           |
|                           |         | 5             | 200                                                                          | 500              | 45             |
| Louisiana,<br>Typical     | <1      | .05           | 8                                                                            | 13               | 3.6            |
|                           |         | .15           | 13                                                                           | 25               | 5              |
|                           |         | .5            | 23                                                                           | 60               | 10             |
|                           |         | 1.5           | 60                                                                           | 150              | 22             |
|                           |         | 5             | 150                                                                          | 300              | 70             |
| Minas,<br>Sumatra         | 0.4-0.7 | .05           | 5-7                                                                          | 9-11             | 2-3            |
|                           |         | .15           | 9-11                                                                         | 19-21            | 3              |
|                           |         | .5            | 22-24                                                                        | 30-53            | 8-9            |
|                           |         | 1.5           | 64-60                                                                        | 128-133          | 20-21          |
|                           |         | 5             | 280-224                                                                      | 360-392          | 70-100         |
| Nigeria,<br>Various       | 0.3-4   | .05           | 4-18                                                                         | 6-28             | 3-11           |
|                           |         | .15           | 8-28                                                                         | 18-44            | 3-13           |
|                           |         | .5            | 21-48                                                                        | 45-84            | 7-19           |
|                           |         | 1.5           | 66-104                                                                       | 120-184          | 21-32          |
|                           |         | 5             | 300-260                                                                      | 300-500          | 120-76         |
| North Slope<br>(Alaska)   | 12-16   | .05           | 36-43                                                                        | 57.6-72          | 31.2-38.4      |
|                           |         | .15           | 54-64                                                                        | 84-96            | 32.4-38.4      |
|                           |         | .5            | 77-104                                                                       | 144-160          | 40.8-51.2      |
|                           |         | 1.5           | 144-168                                                                      | 252-272          | 60-72          |
|                           |         | 5             | 300-336                                                                      | 600-640          | 108-119        |
| Quatar<br>(Midwest)       | 10-20   | .05           | 31-50                                                                        | 50-84            | 26-48          |
|                           |         | .15           | 48-72                                                                        | 50-112           | 28-50          |
|                           |         | .5            | 80-120                                                                       | 120-180          | 34-60          |
|                           |         | 1.5           | 130-190                                                                      | 230-300          | 50-80          |
|                           |         | 5             | 270-360                                                                      | 600-680          | 100-130        |

Table IV-continued

| Crude                      | V(ppm)  | Na Level(ppm) | Dosage for Particular Crude Oils<br>Containing Vanadium at Several Na Levels |         |                |
|----------------------------|---------|---------------|------------------------------------------------------------------------------|---------|----------------|
|                            |         |               | Mg                                                                           | Mg + Si | Additive (ppm) |
| Redwash<br>(Utah)          | <1      | .05           | 8                                                                            | 13      | 3.9            |
|                            |         | .15           | 13                                                                           | 23      | 5              |
|                            |         | .5            | 28                                                                           | 56      | 10             |
|                            |         | 1.5           | 65                                                                           | 150     | 22             |
|                            |         | 5             | 200                                                                          | 40      | 70             |
| Redwater<br>(Canada)       | 0.5-4.5 | .05           | 5.5-19                                                                       | 9-30    | 2-13           |
|                            |         | .15           | 10-30                                                                        | 12-45   | 4-15           |
|                            |         | .5            | 22-50                                                                        | 50-86   | 8-18           |
|                            |         | 1.5           | 65-95                                                                        | 125-180 | 20-30          |
|                            |         | 5             | 250-225                                                                      | 325-495 | 90-770         |
| Smackover<br>(Arkansas)    | <1      | .05           | 8                                                                            | 13      | 3.9            |
|                            |         | .15           | 13                                                                           | 23      | 5              |
|                            |         | .5            | 28                                                                           | 56      | 10             |
|                            |         | 1.5           | 65                                                                           | 150     | 22             |
|                            |         | 5             | 200                                                                          | 40      | 70             |
| Wilmington<br>(L.A. Basin) | 50      | .05           | 100                                                                          | 200     | 125            |
|                            |         | .15           | 185                                                                          | 220     | 125            |
|                            |         | .5            | 200                                                                          | 315     | 130            |
|                            |         | 1.5           | 325                                                                          | 500     | 155            |
|                            |         | 5             | 550                                                                          | 5000    | 220            |

In actually treating one of the fuels mentioned in Table I, approximately 25-30% less additive will be needed than is indicated since there is a significant enrichment of the additive/vanadium ratio during the combustion process. The desired additives can be added as oil soluble materials or dispersions providing homogeneity is achieved.

The silicon content has been found to affect the corrosion rates only slightly and silicon's main function is to provide a more friable and removable slag. The optimum silicon content was determined by means of a simple burner test in which fuel with additive and contaminants (Na, V, S) was atomized into a pilot flame and the combustion products impinge on a metal target

at an appropriate distance in the flame to maintain a temperature of 900°C. This test is described in more detail in the paper "High-Temperature Corrosion in Gas Turbines and Steam Boilers by Fuel Impurities. IV. Evaluation of Silicon and Magnesium-Silicon as Corrosion Inhibitors," to be presented at the American Society of Mechanical Engineers' meeting, Detroit, Michigan, Nov. 1973.

Data from the slag test for Mg-Si and Ca-Al-Si are compared in Tables V and VI. It can be seen from these data that Ca-Al-Si system with Ca/V=0.75, Al/V=2.25 and Si/V=3 forms the most friable and easily removed slag.

Table V

| Na/V | Mg/V | Si/V | Slag Data on Mg-Si with Mg/V=3 and Si/V Varying |                  |                    | Avg. % Lost<br>on Brushing |
|------|------|------|-------------------------------------------------|------------------|--------------------|----------------------------|
|      |      |      | Wt. Deposit                                     | Wt. Deposit/S.A. | % Lost on Brushing |                            |
| 0    | 3    | .1   | 4.5                                             | .86              | 2.23               |                            |
| 0    | 3    | .1   | 6.9                                             | 1.23             | 1.45               |                            |
| .01  | 3    | .1   | 4.1                                             | .77              | 2.44               |                            |
| .01  | 3    | .1   | 5.6                                             | 1.10             | 3.60               |                            |
| .1   | 3    | .1   | 4.6                                             | .82              | 0                  |                            |
| .1   | 3    | .1   | 4.8                                             | .92              | 0                  | 1.13                       |
| 1    | 3    | .1   | 6.4                                             | 1.15             | 0                  |                            |
| 1    | 3    | .1   | 6.0                                             | 1.10             | 1.65               |                            |
| 2.5  | 3    | .1   | 7.3                                             | 1.42             | 0                  |                            |
| 2.5  | 3    | .1   | 3.1                                             | .60              | 0                  |                            |
| 0    | 3    | .2   | 4.8                                             | .92              | 2.1                |                            |
| 0    | 3    | .2   | 5.7                                             | 1.03             | 0                  |                            |
| .01  | 3    | .2   | 4.1                                             | .75              | 2.44               |                            |
| .01  | 3    | .2   | 6.5                                             | 1.20             | 0                  |                            |
| .1   | 3    | .2   | 5.1                                             | .99              | 0                  |                            |
| .1   | 3    | .2   | 6.7                                             | 1.20             | 0                  | 0.44                       |
| 1    | 3    | .2   | 7.5                                             | 1.42             | 0                  |                            |
| 1    | 3    | .2   | 4.4                                             | .85              | 0                  |                            |
| 2.5  | 3    | .2   | 4.0                                             | .74              | 0                  |                            |
| 2.5  | 3    | .2   | 6.7                                             | 1.30             | 0                  |                            |
| 0    | 3    | 1    | 2.0                                             | .384             | 40                 |                            |
| .01  | 3    | 1    | 3.3                                             | .604             | 6                  |                            |
| .1   | 3    | 1    | 5.0                                             | .924             | 10                 | 11.2                       |
| 1    | 3    | 1    | 7.1                                             | 1.31             | 0                  |                            |
| 2.5  | 3    | 1    | 7.2                                             | 1.41             | 0                  |                            |
| 0    | 3    | 2    | 7.0                                             | 1.25             | 20                 |                            |
| .01  | 3    | 2    | 6.6                                             | 1.2              | 20                 |                            |
| .1   | 3    | 2    | 5.4                                             | 1.04             | 20.3               | 12.1                       |
| 1    | 3    | 2    | 6.6                                             | 1.26             | 0                  |                            |
| 2.5  | 3    | 2    | 9.5                                             | 1.73             | 0                  |                            |

Table VI

| Slag Data on Ca-Al-Si |      |      |      |             |                  |                         |
|-----------------------|------|------|------|-------------|------------------|-------------------------|
| Na/V                  | Ca/V | Al/V | Si/V | Wt. Deposit | Wt. Deposit/S.A. | Avg. % Loss on Brushing |
| .01                   | 1.28 | 1.62 | 0.1  | 6.7         | 1.21             | 0                       |
| .1                    | 1.28 | 1.62 | 0.1  | 7.6         | 1.40             | 0                       |
| 1                     | 1.28 | 1.62 | 0.1  | 6.6         | 1.26             | 0                       |
| 2.5                   | 1.28 | 1.62 | 0.1  | 10.4        | 1.85             | 0                       |
| 0                     | .67  | 1.33 | 2    | 8.6         | 1.55             | 29.1                    |
| .01                   | .67  | 1.33 | 2    | 9.7         | 1.76             | 13.4                    |
| .1                    | .67  | 1.33 | 2    | 5.6         | 1.10             | 32.2                    |
| 1                     | .67  | 1.33 | 2    | 6.1         | 1.14             | 1.64                    |
| 2.5                   | .67  | 1.33 | 2    | 9.0         | 1.64             | 0                       |
| 0                     | 1    | 2    | 2    | 5.9         | 1.13             | 20.3                    |
| .01                   | 1    | 2    | 2    | 5.1         | .935             | 31.3                    |
| .1                    | 1    | 2    | 2    | 4.1         | .738             | 19.5                    |
| 1                     | 1    | 2    | 2    | 5.3         | 1.01             | 1.9                     |
| 2.5                   | 1    | 2    | 2    | 6.8         | 1.33             | 0                       |
| 0                     | 1    | 2    | 2    | 4.5         | .87              | 22                      |
| .01                   | 1    | 2    | 2    | 4.0         | .74              | 17.5                    |
| .1                    | 1    | 2    | 2    | 7.8         | 1.49             | 43.6                    |
| 1                     | 1    | 2    | 2    | 7.0         | 1.35             | 0                       |
| 2.5                   | 1    | 2    | 2    | 8.7         | 1.67             | 1.15                    |
| 0                     | .75  | 2.25 | 3    | 9.3         | 1.73             | 62.4                    |
| .01                   | .75  | 2.25 | 3    | 9.0         | 1.61             | 59                      |
| .1                    | .75  | 2.25 | 3    | 6.6         | 1.18             | 60.6                    |
| 1                     | .75  | 2.25 | 3    | 7.5         | 1.36             | 1.3                     |
| 2.5                   | .75  | 2.25 | 3    |             |                  | 36.7                    |

It will be apparent that various changes and modifications may be made in this invention described herein without departing from the scope of this invention. It is intended therefore that all matter contained herein shall be interpreted as illustrative and not as limitative.

What we claim is:

1. A composition of matter consisting essentially of calcium and aluminum in a weight ratio of Ca/Al of about  $\frac{1}{3} \pm 2$  calculated as metal weights.

2. The composition of claim 1 which also contains silicon.

3. The composition of claim 2 where silicon constitutes 1-99% of the composition.

4. The composition of claim 1 where the ratio of Ca/Al is about  $\frac{1}{3}$ .

5. The composition of claim 3 where the ratio of Ca/Al/Si is about 1/1/2 to 1/4/5.

6. A process of inhibiting corrosion in vanadium-containing petroleum fuels which comprises incorporating

25 into said fuels a minor but effective amount of the composition of claim 1.

7. A process of inhibiting corrosion in vanadium-containing petroleum fuels which comprises incorporating into said fuels a minor but effective amount of the composition of claim 2.

8. A process of inhibiting corrosion in vanadium-containing petroleum fuels which comprises incorporating into said fuels a minor but effective amount of the composition of claim 3.

9. A process of inhibiting corrosion in vanadium-containing petroleum fuels which comprises incorporating into said fuels a minor but effective amount of the composition of claim 4.

10. A process of inhibiting corrosion in vanadium-containing petroleum fuels which comprises incorporating into said fuels a minor but effective amount of the composition of claim 5.

\* \* \* \* \*